

## UNITED STATES PATENT OFFICE

EARLE C. PITMAN, OF PRINCETON, NEW JERSEY, ASSIGNOR TO E. I. DU PONT DE NEMOURS & COMPANY, OF WILMINGTON, DELAWARE, A CORPORATION OF DELAWARE

## SOLUBLE NITROCELLULOSE AND COATING COMPOSITION CONTAINING THE SAME

No Drawing.

Application filed January 26, 1926. Serial No. 83,980.

This invention relates to an improved pyroxylin coating composition and the process of preparing the same which involves the modification of the pyroxylin employed to increase its solubility in alcohol. More specifically the nitrocellulose to be employed is modified by digesting nitrocellulose of a nitrogen content not substantially over 11.5% in water at a temperature in excess of 100° C. and under pressure. The resulting product is highly soluble in alcohol and is also a subject of this invention.

One object of the invention is to produce a coating composition of high quality and high viscosity while dispensing with the use of objectionable and high priced solvents.

Another of the objects of the invention is to prepare a nitrocellulose which is substantially completely soluble in a solvent comprising 95% by volume ethyl alcohol. Among the advantages attending the use of a nitrocellulose of this character in the pyroxylin art, is the fact that ordinary denatured alcohol may be employed as a solvent. The use of a cheap, non-poisonous, readily available solvent is thus made practical, where heretofore it has been necessary to resort to the use of solvents of high price or objectionable odor to secure complete solution of the types of nitrocellulose hitherto the most soluble.

The pyroxylin which, up to the development of this process, have had the highest solubility, are those employed in the manufacture of plastics. This type of pyroxylin is generally about 35% soluble in ethyl alcohol denatured with 0.5% by volume of benzol. The rapid decrease in solubility as the strength of alcohol decreases is illustrated in the following table:

Table I

| Strength of alcohol (per cent by volume) | Per cent of nitrocellulose dissolved |
|------------------------------------------|--------------------------------------|
| 100                                      | 100                                  |
| 95                                       | 35                                   |
| 90                                       | 10.5                                 |
| 85                                       | 5                                    |
| 80                                       | 2                                    |
| 60                                       | 0.2                                  |

Table I indicates clearly that there is a wide difference in the character of the most soluble pyroxylin of the prior art which are substantially completely soluble only in 100% alcohol and only 35% soluble in 95% alcohol, and the character of the pyroxylin produced by the present process which are completely soluble in 95% alcohol.

No special type of apparatus is required for carrying out the present process of modification. The digester may be of the ordinary type but should be capable of withstanding an internal pressure of at least 50 pounds per square inch. It should be provided with a steam jacket and suitable safety and relief valves. Since some acidity is likely to be developed in the process, the digester should be constructed of material not readily corroded by dilute nitric and sulphuric acids at the temperatures of digestion.

In carrying the process into effect the digester is partly filled with water and the nitrocellulose is then added. It is important to note that the pyroxylin should always be kept in a wet condition to avoid danger of rapid decomposition or explosion. I prefer to use an amount of water sufficient to completely cover the nitrocellulose but a much greater amount of water is not objectionable, except, perhaps, economically. After charging, the digester is closed and the charge heated under pressure. The time required for completion of the operation, in general, is less the higher the temperature of digestion. In this connection it may be remarked that it would appear that temperatures below 110° C. are impracticable commercially because of the slowness of the operation, while temperatures above 140° C. are undesirable because of the danger of rapid decomposition. The time required to attain complete solubility at a given temperature will vary with the nature of the starting material but, in general, will be between 3 and 30 hours.

In the course of the digestion some gas is generated. This is especially noticeable at temperatures above 135° C. As this gas is not readily dissolved in water, it is desirable to eliminate it by occasionally open-

ing the relief valve. Digestion is continued until the product becomes more than 99% soluble in denatured alcohol containing 95% ethyl alcohol.

5 It will be evident that conditions of operation, materials employed, etc., may be varied within a wide range. This is illustrated in the following table, wherein are set forth the limits within which I have 10 found the best results are obtained together with the specific conditions preferable for our purposes. It is to be understood, however, that obvious departures from the ranges therein specified to adapt our process to peculiar conditions are entirely within the 15 scope of the invention.

Table II

|                                                         | Range     | Preferred |
|---------------------------------------------------------|-----------|-----------|
| Temperature of digestion (°C.)                          | 110-140   | 130       |
| Per cent nitrogen content of nitrocellulose used        | 10.5-11.5 | 11.0      |
| Per cent alcohol soluble content of nitrocellulose used | 20-60     | 30        |
| 25 Ratio of water to dry nitrocellulose                 | 0.5/1-    | 10/1      |

Although denatured alcohol soluble products may be prepared from pyroxylins of 30 lower than 10.5% nitrogen content and more than 60% initial solubility I have not included them, since their high solubility in the nitrating acids and their tendency to disintegrate during manufacture render 35 them unfeasible as raw materials for a commercial process. Likewise, I estimate that temperatures below 110° C. are impractical commercially, merely because of the slowness of the operation and that temperatures above 40 140° C. are undesirable because of the danger of rapid decomposition.

The soluble nitrocellulose of my invention is substantially undergraded, as is indicated by stability tests of at least 30 minutes. 45 These tests were made according to the German method (see "Nitrocellulose Industry", Worden, 1911, page 971).

It also shows a viscosity of from 10 to 300 centipoises at 28° C. when tested in the form 50 of a 6.5% nitrocellulose solution in amyl acetate.

In order to further illustrate the process by which the soluble nitrocellulose is produced, the following typical embodiments of 55 the process are furnished:

Example A

60 24.2 lbs. of stabilized nitrated paper containing 30% moisture was immersed in 30 gallons of water in a 50 gallon steam jacketed digester and heated under pressure continuously for 6 hours at a temperature of 131°- 65 134° C. The product was washed in water.

The initial and final properties were as follows:

|                                                                           | Original   | Final  | 70 |
|---------------------------------------------------------------------------|------------|--------|----|
| Nitrogen content                                                          | 10.94%     | 10.60% |    |
| German test (minutes)                                                     | 60         | 35     |    |
| Viscosity at 25° C. (6% nitrocellulose in 30% camphor-alcohol by wt.)     | 1,855 cp.  | 30 cp. |    |
| Viscosity at 28° C. (6.5% nitrocellulose in amyl acetate)                 | 89,200 cp. | 28 cp. |    |
| Per cent soluble in denatured alcohol (95% ethyl alcohol and 0.5% benzol) | 22.9       | 100.0  | 75 |

Example B

302 g. of stabilized nitrated linters containing about 35% moisture was immersed in 2340 g. of water in a 1 gallon steam jacketed autoclave and heated under pressure continuously for 9 1/4 hours at 127°-131° C., the gauge pressure varying from 28 lbs. to 32 lbs. The product was washed in water. 80

The initial and final properties were as follows:

|                                                                           | Original       | Final          | 90 |
|---------------------------------------------------------------------------|----------------|----------------|----|
| Nitrogen content                                                          | Per cent 11.05 | Per cent 10.71 |    |
| Viscosity at 28° C. (6.5% nitrocellulose in amyl acetate)                 | (*)            | 18             |    |
| Per cent soluble in denatured alcohol (95% ethyl alcohol and 0.5% benzol) | 43.2           | 100.00         | 95 |

\* Viscosity not run in amyl acetate because of poor solubility. Viscosity of 6% solution of nitrocellulose in 30% camphor denatured alcohol (by weight) 1589 cp. at 25° C.

The above examples indicate that the digestion must be more severe in the case of nitrated linters than in the case of nitrated paper. 100

In the above examples 95% ethyl alcohol containing 0.5% benzol was employed as the solvent of the product in both cases. Tests have indicated, however, that the presence of 105 0.5% benzol as a denaturant in 95% by volume ethyl alcohol has so slight an effect on the solubility of the nitrocellulose as to be negligible for all practical purposes.

In all cases the solubility of the nitrocellulose in alcohol was determined by the following method: Shake 1 gram nitrocellulose in 200 cc. of alcohol for two hours. Filter on a weighed Gooch. Dry Gooch and determine the weight of the insoluble residue. The excess of alcohol is so great that it can be assumed the portion of nitrocellulose insoluble in it would not be dissolved in any amount of alcohol of the same concentration. 110

The soluble nitrocellulose is peculiarly adapted for incorporation into a pyroxylon enamel or lacquer. By reason of its extreme solubility in ethyl alcohol it is possible to employ ordinary denatured alcohol in place of more expensive or otherwise objectionable solvents heretofore used in the preparation of such compositions. 125

In order to present in detail the nature of 130

the improved coating compositions made from the solubilized nitrocellulose, typical examples are given below. It is to be understood that these are entirely illustrative of the invention.

Following is an example of a coating composition in which the use of alcohol-soluble nitrocellulose makes it possible to eliminate ethyl acetate:

10

*Example C*

|                                    | Prior art | New      |
|------------------------------------|-----------|----------|
|                                    | Per cent  | Per cent |
| Pyroxylin (12% N)                  | 10        | 14       |
| Pyroxylin (soluble in 95% alcohol) |           |          |
| Castor oil                         | 20        | 10       |
| Pigment                            | 15        | 14       |
| Ethyl acetate                      | 30        | 30       |
| Benzol                             | 15        | 14       |
| Denatured alcohol (95% by vol.)    | 100       | 100      |

An example of a high solids enamel of the new type is given below. It will be noted that the ethyl acetate of the prior art enamel has been replaced by ethyl alcohol and the butyl acetate by diethyl carbonate, making the odor of the new type enamel unobjectionable for interior use:

30

*Example D*

|                                         | Prior art | New      |
|-----------------------------------------|-----------|----------|
|                                         | Per cent  | Per cent |
| Pyroxylin (11.5%-12.5% N)—low viscosity | 8         | 8        |
| Pyroxylin (soluble in 95% alcohol)      |           |          |
| Pigment                                 | 6         | 6        |
| Ester gum                               | 6         | 6        |
| Tricresyl phosphate                     | 4         | 4        |
| Toluol                                  | 27        | 27       |
| Xylool                                  | 7         | 7        |
| Ethyl acetate                           | 12        | 17       |
| Denatured alcohol (95% by vol.)         | 5         | 5        |
| Butyl alcohol                           | 20        | 20       |
| Diethyl carbonate                       |           |          |
| Butyl acetate                           |           |          |
|                                         | 100       | 100      |

The compositions given above are on the basis of spraying consistency. The proportion of pigment will, of course, vary according to the hiding power and other properties of the pigment, being as low as two parts in the case of some black enamels and as high as 25 parts for some light colors, such as whites.

The use of pyroxylin soluble in denatured alcohol is also of advantage in the so-called mixing lacquers, which are solutions of nitrocellulose, usually in cheap solvents, added to solutions of shellac in such a solvent as denatured alcohol. The purpose of introducing the nitrocellulose is to waterproof the shellac, which is well known to be highly permeable to water.

Following are illustrations of the use of alcohol-soluble nitrocellulose in mixing lacquers.

*Example E*

|                                                   | Prior art | New      |     |
|---------------------------------------------------|-----------|----------|-----|
|                                                   |           | (A)      | (B) |
| Pyroxylin (11.5% N)                               | 8         | Per cent | 70  |
| Pyroxylin (soluble in 95% alcohol)                |           | 20       | 15  |
| Ethyl acetate                                     | 32        |          |     |
| 95% ethyl alcohol (denatured with methyl alcohol) | 32        | 43       | 85  |
| Toluol                                            | 28        | 37       |     |
|                                                   | 100       | 100      | 75  |
|                                                   |           | 100      |     |

Formula (B) is no cheaper than (A), but may be used where the presence of toluol is objectionable.

In order to effect the waterproofing of the shellac, mix 100 parts of the prior art lacquer, or 50 parts of the new type of lacquer, with 100 parts of a solution of 30% by weight of shellac in ethyl alcohol denatured with 10% methyl alcohol. In addition to the saving enabled by the use of a cheaper solvent mixture the higher solids content of the new lacquer at the same viscosity reduces the total amount of solvent which must be evaporated to deposit a given weight of coating.

Tests have shown the films produced by the coating composition in which the modified nitrocellulose and denatured alcohol are employed to be equal in quality, viscosity and durability to those produced from the unmodified types of nitrocellulose with the more expensive and objectionable solvents formerly employed.

I claim:

1. The method of treating cellulose nitrate comprising digesting cellulose nitrate at elevated pressure in a non-solvent, inert liquid at a temperature above 100° C. and below the decomposition point of the cellulose nitrate, and stabilizing the product by washing with water.

2. The method of treating cellulose nitrate comprising digesting cellulose nitrate in water at a temperature between 110° C. and 140° C. at a pressure above atmospheric and below about 50 pounds per square inch and washing with water to produce a stability of thirty minutes (German test).

3. A cellulose nitrate of reduced viscosity having a nitrogen content of at least 10% and less than 11.5% and being substantially completely soluble in 95% ethyl alcohol and having a stability of thirty minutes (German test).

4. A cellulose nitrate of reduced viscosity showing a stability of at least 30 minutes (German test) and being more than 99% soluble in 95% ethyl alcohol.

5. The method of making a cellulose nitrate having about 99% solubility in 95% ethyl alcohol comprising digesting cellulose nitrate having a nitrogen content between about 10% and 11.5% in an inert non-solvent

80

85

90

95

100

105

115

120

125

130

liquid at pressure above atmospheric and at a temperature above 100° C. but below the decomposition point of the cellulose nitrate and washing with water until the product is stable.

6. The method of making a cellulose nitrate having 99% solubility in 95% ethyl alcohol comprising digesting cellulose nitrate having a nitrogen content between about 10% and 11.5% in water at pressure above atmospheric but less than about 50 pounds per square inch and at a temperature between 110° C. and 140° C. until 99% solubility in 95% ethyl alcohol is obtained and stabilizing 10 by washing with water until the product will 15 give a German test upward of about thirty minutes.

7. The method of making a cellulose nitrate having 99% solubility in 95% ethyl alcohol 20 comprising digesting a cellulose nitrate having a nitrogen content between about 10% and 11.5% in water at a pressure of about 20-40 pounds per square inch, and at a temperature between 100° C. and 140° C. and in 25 stabilizing the digested cellulose nitrate by washing with water until it will give a German test of at least thirty minutes.

8. A coating composition comprising a solution of a cellulose nitrate of reduced viscosity having a nitrogen content between 10% and 11.5%, a stability of thirty minutes (German test), and which is substantially completely soluble in 95% ethyl alcohol.

In testimony whereof I affix my signature.  
35 EARLE C. PITMAN.

40

45

50

55

60

65